

July 6, 1937.

J. V. VAUGHEN

2,085,776

CADMUM ELECTRODEPOSITION

Filed Oct. 17, 1935



INVENTOR.

JOHN V. VAUGHEN.

BY

*Albert B. Briggs.*

ATTORNEY.

## UNITED STATES PATENT OFFICE

2,085,776

## CADMIUM ELECTRODEPOSITION

John V. Vaughn, Lakewood, Ohio, assignor, by  
mesne assignments, to E. I. du Pont de Ne-  
mours & Company, Wilmington, Del., a corpo-  
ration of Delaware

Application October 17, 1935, Serial No. 45,391

17 Claims. (Cl. 204—1)

This invention relates to the electrodeposition of cadmium from cyanide-cadmium baths, and is particularly directed to cyanide-cadmium plating compositions, plating baths, and plating processes which employ, as an addition agent, a ketaldone-amine reaction product whereby a bright, smooth, uniform cadmium deposit is obtained.

It has heretofore been proposed to modify the character of cadmium deposits by the use of organic addition agents such as sulfite cellulose waste, dextrin, starch, alkylated naphthalene sulfonic acids, wool, caffeine, shellac, casein, licorice, glucose, alkali reaction products of heterocyclic aldehydes, furfural gum arabic, and gelatine.

It has been necessary to employ an addition agent and/or a brightener with cyanide-cadmium plating baths, because, without such modifying agents, cadmium deposits of exceedingly poor character and appearance are obtained. The properties of electrodeposited cadmium are largely determined by the addition agent and/or brightener used, and the desirability of a cadmium plate is, to a great extent, dependent upon the efficacy of the modifying agents employed.

The properties of a cadmium plate are partly dependent, in commercial practice, upon certain characteristics of the plating bath employed, and these characteristics can be modified, to some extent, by suitable organic addition agents and/or brighteners. Under strictly controlled conditions, one can deposit a fairly satisfactory cadmium plate on a flat cathode with a bath which, in ordinary commercial practice, would be unsatisfactory. Under the usual conditions of commercial operation, particularly when recessed articles or articles of irregular shape are to be plated, a bath must have a fairly wide bright current density range and good throwing power if even moderately satisfactory results are to be obtained. The throwing power and the extent of the bright range have been somewhat improved by the use of the addition agents heretofore known.

While the addition agents hitherto employed have effected a considerable improvement in processes for the electrodeposition of cadmium, the results obtained have not been all that could be desired.

I have found that amine derivatives of ketaldones are exceedingly effective addition agents for cyanide-cadmium plating. By the use of these novel addition agents, it is possible to electrodeposit cadmium from cyanide-cadmium baths as a bright, smooth, lustrous, ductile, adherent

deposit. Baths containing these novel addition agents are characterized by good throwing power and by a wide bright current density range.

In the accompanying drawing there are shown the relationships existing between various derivatives which constitute the addition agents of my invention, and there are also shown, diagrammatically, the methods of preparation of the various derivatives.

Represented by a circle in the upper left-hand corner of the drawing are the starting materials from which my addition agents are derived. The starting materials are designated "ketaldones" but, as will become apparent hereinafter, the best results are obtained by the use of certain aliphatic and carbocyclic aldehydes and ketones.

I have applied the term "ketaldonyl" to designate the  $\text{C}=\text{O}$  group as it appears in aldehydes and ketones in contradistinction to the  $\text{C}=\text{O}$  group as it appears in acids. Of course, the carbonyl group as it appears in acids,



5

15

25

30

35

40

45

is very different in its properties from the carbonyl group as it appears in aldehydes and ketones, and the expression "ketaldonyl group" is employed to distinguish the aldehydic and the ketonic carbonyl group from the acidic carbonyl group. The expression "ketaldonyl group" as used herein designates a carbonyl group in which a third carbon valence is joined to carbon and in which the remaining valence is satisfied by carbon or by hydrogen. Or, in chemical symbols, the "ketaldonyl group" as used herein is of the type



wherein R is a hydrocarbon radical and wherein R' is hydrogen, in the case of an aldehyde, or R' is a hydrocarbon radical, in the case of a ketone. It will also be understood that the ketones and aldehydes themselves are referred to herein as ketaldones in accordance with this terminology.

The starting materials which I employ are, broadly, ketaldones. While I may use aldoses, 50 ketoses, heterocyclic aldehydes and ketones or any other such ketaldones, I prefer to use aliphatic and carbocyclic ketaldones which do not contain a carboxyl group, which do not contain sulfur, and which do not contain nitrogen. The 55

starting materials, moreover, should contain no more than two hydroxyl groups and preferably should contain at least two carbon atoms. More specifically, I prefer to employ ketaldones which contain only carbon, hydrogen, and oxygen, which contain at least two carbon atoms, and in which the hydrogen-oxygen ratio is greater than that of water.

As is illustrated in the drawing, the starting materials, the ketaldones, are reacted with an amine, in alkaline solution, to produce a ketaldone-amine reaction product.

A preferred group of ketaldones, the aldacet, are illustrated in the upper right-hand corner of the drawing. More will be said hereinafter regarding the members of the illustrated aldacet equilibrium. As is shown in the drawing, the aldacet, like the ketaldones generally, are reacted with an amine to produce a ketaldone-amine reaction product.

The aldacet comprise the aliphatic aldehydes: acetaldehyde, aldol, crotonaldehyde, and paraldehyde. In dilute alkaline solution the aldacet appear to exist in equilibrium, any one of the aldacet leading to the production of all at a rate of conversion apparently depending upon the specific aldacet first present. The aldacet equilibrium is illustrated in the upper, right corner of the drawing.

Referring to the aldacet equilibrium in more detail, it is noted that acetaldehyde in dilute alkaline solution is quickly converted to aldol thus:



The aldol may lose one molecule of water and become crotonaldehyde, thus:



The aldol may condense to form paraldehyde, thus:



The  $n$  in Equation 3 is a whole number, probably 2.

In order to visualize the relationships existing between the aldacet, reference should be had to the accompanying drawing wherein these relationships are diagrammatically illustrated. It is to be understood that the relationships are shown with reference to the compounds in dilute alkaline solutions.

In the drawing, acetaldehyde is illustrated as converting to aldol. The aldol may go to paraldehyde or to crotonaldehyde. The aldol might also go back to acetaldehyde, but only to a small extent. The paraldehyde may go back to aldol, or it may lose water and go to crotonaldehyde, though this latter conversion probably takes place to a very small degree. The crotonaldehyde may form from acetaldehyde, aldol, or paraldehyde, and, by gaining water, may revert to any of them, though it is likely that it would move largely by way of aldol.

As is seen in the drawing, then, we may consider the aldacet as being in equilibrium. This equilibrium will, according to my belief, be substantially the same regardless of which of the four substances are initially added to the cyanide solution, though, as will hereinafter be noted, the aldacet are not entirely equivalent and it is possible that some of the aldacet in dilute alkaline

solution form this aldacet equilibrium rather slowly or move more rapidly in certain directions than in others.

While I have mentioned only acetaldehyde, aldol, crotonaldehyde, and paraldehyde as members of this sub-genus, I may use any condensation product of acetaldehyde in dilute alkaline solution. Another aldacet is paraldehyde. Ordinarily paraldehyde is considered as forming only in acid solutions, but I have reason to believe that at least some paraldehyde forms in the discussed aldacet equilibrium. Paraldehyde is apparently very slow to convert to other aldacet and probably because of this fact is none too satisfactory a starting material.

Aldol, acetaldehyde, crotonaldehyde, and paraldehyde are the only commercially available aldacet at the present time. For practical reasons, therefore, I prefer to use as a starting material, an aldehyde selected from the group consisting of acetaldehyde, aldol, crotonaldehyde, and paraldehyde.

It is to be noted that the aldacet are those aliphatic ketaldones, such as acetaldehyde, aldol, crotonaldehyde, and paraldehyde, which exist in some sort of equilibrium when one of the said ketaldones is put into alkaline solution. Generally, then, one might say that the aldacet are aliphatic aldehydes from the group consisting of acetaldehyde and its equilibrium products in alkaline solutions. It will be understood that the aldacet include the equilibrium products as above described, and that they do not include irreversible condensation products which may not reversibly lead to the formation of the aldacet equilibrium.

As a definition for the purposes of this application, then, the aldacet are reversible equilibrium-condensation products of acetaldehyde in alkaline solution, and particularly in alkaline solutions such as those of the following Example I.

As will be noted in detail hereinafter, the aldacet are not entirely equivalent for my purposes but are substantially so. Crotonaldehyde, for example, seems to lead to slightly lower yields. This may be attributable to the fact that crotonaldehyde is but slowly converted to the necessary form, or to some other now unknown cause.

As is above mentioned, there is considerable uncertainty as to the extent and nature of the conversion of some aldacet to others. All of the evidence now available to me substantiates the putative theory above advanced as to the nature of the aldacet equilibrium, but it will be understood that direct experimental evidence is obtainable only with great difficulty. In most instances the aldacet equilibrium exists for only a short time, some further action quickly taking place to form resins. That the aldacet are in some kind of equilibrium is relatively certain, but the proportions of individual aldacet and the rates of conversion have, to date, defied exact determination.

It is clearly to be understood that the above description of the relations between the initial materials is for purposes of illustration and that I do not intend to be limited in any way thereby, because the chemistry of these compounds is intricate and obscure, and because my results are obtained entirely apart from theoretical considerations. It is also to be understood that while I refer to aldol, acetaldehyde, crotonalde-

hyde, and paraldol as resulting from the condensation of acetaldehyde in alkaline solutions, I do not wish to be limited thereby, as I may use aldol, acetaldehyde, crotonaldehyde, and paraldol which have been made in any manner.

Turning now to a consideration of the ketaldone-amine reaction products produced from the aldacet, it is first noted that the term "reaction" is used to express whatever occurs when the ketaldones, or specifically the aldacet, are treated with an amine. The term "reaction" is used to distinguish from "condensation" as used above with reference to the aldacet equilibrium tho, in fact, the reaction probably includes both polymerizations and condensations.

The reaction which leads to the aldacet-amine reaction products takes place, I believe, between amine and one or more of the aldacet. This reaction is illustrated in the drawing by dashed lines. The aldacet, or aldacet, which react with the amine may go first to some other and unknown form and then react. I conceive of the reaction as withdrawing one, or more, of the aldacet from the equilibrium with the result that the remaining aldacet move towards the removed materials to restore the equilibrium, and are so all finally utilized.

To illustrate the production of the addition agents of my invention, the following specific examples are given:

#### EXAMPLE I

Equimolecular proportions of crotonaldehyde and monoethanolamine were reacted, starting the reaction at room temperature. The temperature of the mixture was held at about forty to fifty degrees centigrade until no further reaction was apparent. The reaction mixture was a reddish-brown, viscous liquid, readily soluble in cyanide-cadmium plating baths.

The addition agent of this example was employed as an addition agent in a cyanide-cadmium bath made up as follows:

| Bath (1)                                              |     | Grams per liter |
|-------------------------------------------------------|-----|-----------------|
| Sodium cyanide (NaCN)                                 | 130 |                 |
| Cadmium oxide (CdO)                                   | 43  |                 |
| Sodium sulfate (Na <sub>2</sub> SO <sub>4</sub> )     | 50  |                 |
| Cobalt sulfate (CoSO <sub>4</sub> ·7H <sub>2</sub> O) | 10  |                 |
| Addition agent                                        | 1.2 |                 |

A plating solution was made up and used in the customary way to plate a number of articles with a cadmium deposit about five-thousandths of an inch thick. After washing with water, the articles were examined and found to have a perfectly smooth, mirror-like finish. It is, of course, very difficult with prior art processes to obtain even a fairly smooth finish when so thick a deposit of cadmium is plated.

The bath of this example displayed good throwing power and a wide bright current density range.

The product of this example may satisfactorily be employed in widely varying amounts, but I usually prefer to use between about eight-tenths and two grams per liter. The proportion of the agent used above, one and two-tenths grams per liter, is about an optimum under the conditions of this example.

The following specific example illustrates the use of the product of this example as an addition agent in a dilute bath:

| Bath (2)              |     | Grams per liter |
|-----------------------|-----|-----------------|
| Cadmium oxide (CdO)   | 26  |                 |
| Sodium cyanide (NaCN) | 87  |                 |
| Addition agent        | 0.7 | 5               |

This bath was used for plating several objects at a current density of twenty amperes per square foot. The deposit was extremely bright and smooth. The number of grams of cadmium oxide in the above bath may be varied between fifteen and thirty-five and good results will be obtained. If the bath be too concentrated the deposit will not be entirely satisfactory.

The addition agent is used in about an optimum proportion for the conditions of this example, but I may advantageously employ from about five-tenths to about seventy-five hundredths gram per liter of this agent.

While my addition agents are effective in any customary cyanide bath, I prefer to use baths of the kind set forth in U. S. Patent 1,681,509 to Mr. Leon R. Westbrook, and in Bath (1). These baths are of the cyanide type, and contain a small amount of a compound of a metal of the iron group having an atomic weight greater than fifty-eight. The details as to the formulation and use of these baths may be found in the said Patent 1,681,509 and need not be duplicated here.

The plating baths of the said Patent 1,681,509 are modified only by employing my novel addition agents in lieu of the addition agents, goulac, dextrin, starch, etc., mentioned therein. While the plating processes described in the said Patent 1,681,509 lead to a bright, hard, dense, and smooth deposit of cadmium, and while the invention therein described and claimed has been widely accepted by the art because of its merit, the substitution of my addition agents for those in the patent results in a cadmium deposit of even greater smoothness, uniformity, and brightness.

Of course, I may use other compounds of metals of the iron group having an atomic weight greater than fifty-eight, such as nickel, copper, etc., as disclosed in the heretofore mentioned Patent 1,681,509, but the use of cobalt compounds, as in Bath (1), has led to the best results.

I desire that it be clearly understood that the whole disclosure of the heretofore mentioned Patent 1,681,509, as well as that of U. S. Patent 1,564,413 to Clayton M. Hoff, cited therein, is to be considered, in its entirety, as an integral part of my disclosure, as my novel addition agents co-act with the cyanide-metal compound baths therein to produce a result unexpected from an examination of the attributes of either my addition agents or the baths of the said patent.

While I have discussed above the use of baths of the Westbrook type, I do not wish to be limited thereto. I prefer to use them because of certain commercial considerations, and because they may be more concentrated, but excellent results are obtainable with other types of baths, such as Bath (2) above.

#### EXAMPLE II

A reaction product similar to that of Example I was produced by reacting equimolecular proportions of aldol and monoethanolamine. A product exceedingly similar to the one of Example I was produced, and comparable results were obtained when the product of this example was

used as an addition agent in cyanide-cadmium plating baths of the type shown in Example I.

#### EXAMPLE III

- 5 One-half mole of monoethanolamine and one mole of aldol were reacted at temperatures between 30 and 40° C. The product was not as soluble as the product of Example II, and it was not as satisfactory an addition agent for use in cyanide-cadmium plating.

#### EXAMPLE IV

- Equimolecular proportions of aldol and diethanolamine were reacted to room temperatures. 15 A product very similar to those of the above examples was produced, the product of this example, however, being slightly less soluble than the product of Examples I and II.

The product of this example and some of the hereinafter mentioned products are not readily soluble in cyanide-cadmium plating baths, and it is desirable that they be dispersed in the baths. It is expedient to disperse the addition agent if difficulty is encountered in dissolving an optimum 25 quantity. The addition agents may be dispersed and their dissolution aided by adding them to a cyanide-cadmium bath in a suitable solvent, such as alcohol or acetone. It may sometimes be found desirable to reduce the addition agents to a finely divided state, or to use them in conjunction with such dispersing agents as saponin, gum arabic, and sulfite cellulose waste.

#### EXAMPLE V

Equimolecular proportions of aldol and triethanolamine were reacted at room temperatures. The reaction product of this example was somewhat less soluble than the products of Examples I and II. While the product of this example 40 caused the production of a very bright deposit when added to a cyanide-cadmium plating bath, the bath had a more restricted bright current density range than when the products of Examples I and II were used.

While I have shown the reaction of the aldacet with certain amines in the above examples, it will be understood that other amines may be used. I may, for instance, prepare addition agents by 45 treating the aldacet with amines such as the glucamines, for instance, glucamine and methyl glucamine, or aliphatic amines, for instance, methyl ethylamine, methylamine, and ethylamine.

While the aldacet-amine reaction products 55 may be prepared by conducting the reactions of the above examples at rather widely varied temperatures, I prefer that the reaction be performed at temperatures between about thirty and fifty degrees centigrade. If much lower temperatures be maintained, the reaction products 60 will tend to contain insoluble or relatively inactive constituents. Similarly, the reaction temperatures should not be permitted to rise too high, because, when the reaction proceeds at high 65 temperatures, the reaction product may contain insoluble constituents and may have none too great an efficiency as an addition agent.

It is generally preferred to employ an equimolecular proportion, or an excess, of amine to aldehyde. As will be noted by comparing Examples 70 II and III, less satisfactory amaldacets are produced when less than an equivalent amount of amine is used.

In the foregoing, the products derived by 75 reacting an aldacet with an amine have been dis-

cussed in some detail with reference to their preparation, their properties, and their applications as addition agents in cyanide-cadmium plating. The products thus considered above are, in many respects, typical of the addition agents 5 of my invention.

The above products are, of course, derived from certain aliphatic ketaldones: the aldacets. Below are discussed typical ketaldone-amine reaction products derived from other aliphatic ketaldones 10 and from carbocyclic ketaldones.

The following typical aliphatic ketaldones were tried as starting materials for the production of addition agents. The aldacets are included for purposes of comparison. The compounds in the respective lists are given in about 15 the order of their desirability as starting materials.

#### Aldehydes

|                                             |    |
|---------------------------------------------|----|
| 1. Aldol                                    | 20 |
| 2. Acetaldehyde                             |    |
| 3. Crotonaldehyde                           |    |
| 4. Paraladol                                |    |
| 5. Propionaldehyde                          | 25 |
| 6. $\alpha$ -ethyl $\beta$ -propyl acrolein |    |
| 7. Butyraldehyde                            |    |
| 8. Acrolein                                 |    |
| 9. Citral                                   |    |
| 10. Citronellal                             | 30 |
| 11. Hexadecenoic aldehyde                   |    |
| 12. Isobutylaldehyde                        |    |

#### Ketones

|                                   |    |
|-----------------------------------|----|
| 1. Diethyl ketone                 | 35 |
| 2. Methyl <i>n</i> -propyl ketone |    |
| 3. Methyl ethyl ketone            |    |
| 4. Diacetyl                       |    |
| 5. Light acetone oil              |    |
| 6. Heavy acetone oil              | 40 |
| 7. Isobutyl ketone                |    |
| 8. Acetone                        |    |
| 9. Iso amyl ketone                |    |

Considering more specifically the preparation of addition agents from the above aliphatic ketaldones, the following specific examples are given to illustrate the mode of production:

#### EXAMPLE VI

Equimolecular proportions of monoethanolamine and propionaldehyde were reacted at room temperature. A soluble resin was obtained which, when employed in baths such as those of Example I, displayed activity as an addition agent but was none too satisfactory.

#### EXAMPLE VII

Methyl ethyl ketone was treated at about 40° to 50° C. with diethanolamine in equimolecular proportions. The resulting reaction product displayed activity as an addition agent in cyanide-cadmium plating baths.

When aliphatic ketaldones are used as starting materials, a ketaldone should be selected which contains at least two carbon atoms. Formaldehyde, with but one carbon atom, stands in a unique position with respect to aldehydes generally. Its dissimilarity to the other aldehydes is, of course, generally recognized, and it does not lead to the production of entirely satisfactory addition agents.

In view of the difference between formaldehyde and other aldehydes, one would expect formaldehyde to behave differently as a starting material for the production of addition agents.

As addition agents prepared from formaldehyde are of a different order of effectiveness and are of a different character from the agents prepared from other aldehydes, I prefer to employ 5 ketaldones which have more than one carbon atom.

As the aliphatic ketaldones contain more and more carbon atoms, they appear to become less desirable as starting materials for the production 10 of amketaldoresins. Citral and citronellal, for example, with nine carbon atoms are quite satisfactory as starting materials for the production of addition agents, but the agents tend to be somewhat insoluble. They may, of course, be dispersed in the bath, but it is ordinarily preferable that the agents be readily soluble in the amounts required.

Above about nine carbon atoms the aliphatic ketaldones become somewhat less desirable as 20 starting materials. Hexadecalaldehyde, for instance, with sixteen carbon atoms led to the production of a relatively insoluble, though operative, product. I prefer, accordingly, to employ aliphatic ketaldones containing between two and 25 nine carbon atoms. This terminology includes acetraldehyde, for example, as a two carbon atom compound and citral as a nine carbon atom compound. I especially prefer to employ those aliphatic ketaldones of two to nine carbon atoms 30 which contain no more than two hydroxyl groups.

I have found that it is not desirable that the aliphatic ketaldones contain carboxyl groups. Moreover, the elements sulfur and nitrogen are 35 preferably absent from the aliphatic ketaldones which I employ as starting materials for the production of my addition agents. I especially prefer to use aliphatic ketaldones which contain only carbon, hydrogen, and oxygen, and in which the hydrogen-oxygen ratio is higher than that of 40 water.

While, as is above noted, I prefer that the aliphatic ketaldones which I employ as starting materials contain no more than two hydroxyl groups, and, more specifically, that they have a higher ratio of hydrogen to oxygen than that of 45 water, it is, nevertheless, within the scope of my present invention to use such ketaldones as ketoses and aldoses.

When carbohydrates which contain an aldehyde or ketone group are treated with an amine, products similar to those above may, with some difficulty, be prepared. The products thus produced, however, are of a different order of effectiveness from the preferred products.

The products prepared from the aliphatic ketaldones have been discussed above in some detail, and it is now proposed to discuss briefly the preparation of ketadone-amine reaction products from carbocyclic ketaldones.

The following carbocyclic ketaldones, tried as starting materials for the production of ketadone-amine products, are listed in the approximate order of their desirability.

1. Cyclohexanone
2. Methyl cyclohexanone
3. Benzoin
4. Benzaldehyde
5. Anisic aldehyde
6. Cinnamic aldehyde
7. Quinone
8. Vanillin
9. Ortho-ortho dicarboxy benzoin

In order more fully to describe the production of addition agents from the carbocyclic ketaldones, the following illustrative example is given:

#### EXAMPLE VIII

Equimolecular proportions of monoethanolamine and benzaldehyde were reacted at about 40° to 50° C. The product displayed activity as an addition agent in cyanide-cadmium plating baths of the types shown in Example I.

The other carbocyclic compounds above listed may be similarly treated with an amine according to the above procedures with good results.

While generally I may advantageously employ any carbocyclic ketadone, I prefer to use as starting materials ketaldones which do not contain a carboxyl group and which do not contain sulfur. Moreover, carbocyclic ketaldones which do not contain nitrogen are ordinarily preferred, because while Michler's ketone, for instance, responds to my broadest definition, it is none too satisfactory a starting material. Specifically, I prefer to employ carbocyclic ketaldones which contain only carbon, hydrogen, and oxygen and in which the hydrogen-oxygen ratio is greater than in water.

The foregoing discussion of the aromatic ketaldones is limited to a preferred group, the carbocyclic ketaldones. It will be understood, however, that my invention in its broad aspects includes the use of cyclic ketaldones generally. I may, for instance, use heterocyclic ketaldones, such as furfural, as starting materials for the preparation of addition agents for cyanide-cadmium plating baths.

In order conveniently to merchandise my novel addition agents, I may incorporate them with the dry ingredients employed to make up a plating bath. The resulting dry mixture can then be packaged and sold to the consumer who needs only to dissolve the mixture in water for use. Again, I may find it desirable to incorporate the addition agent with only one or a few of the ingredients and let the consumer add the other 35 ingredients. Frequently, of course, it will be desirable to merchandise the novel addition agents as such.

While I have disclosed a number of specific cyanide-cadmium baths heretofore, it will be 45 understood that I do not intend to be limited thereby and that the teachings of my invention may be applied to cyanide-cadmium baths generally.

It will be also understood that I do not intend to be limited to the specific ketadone-amine reaction products above disclosed, as numerous other such compositions can readily be prepared by those skilled in the art according to the principles of my invention.

I claim:

1. A cyanide-cadmium plating composition containing an amine reaction product of a ketadone.
2. A cyanide-cadmium plating composition containing an amine reaction product of a carbocyclic ketadone.
3. A cyanide-cadmium plating composition containing an amine reaction product of an aliphatic ketadone.
4. A cyanide-cadmium plating composition containing an amine reaction product of an aliphatic ketadone which contains only carbon, hydrogen and oxygen, which has no less than two and no more than nine carbon atoms, and in which the ratio of hydrogen to oxygen is greater than that of water.
5. A cyanide-cadmium plating composition containing an amine reaction product of an aldaacet, an aldacet being, as herein set forth, one of

5

10

15

20

25

30

35

40

45

50

55

60

65

70

75

the aldehyde equilibrium products which results when acetaldehyde is put in alkali metal cyanide solution.

6. A cyanide-cadmium plating composition containing an amine reaction product of an aliphatic aldehyde selected from the group consisting of aldol, acetaldehyde, crotonaldehyde, and paraldol.

7. A cyanide-cadmium plating composition containing an amine reaction product of aldol.

8. A cyanide-cadmium plating composition containing an ethanolamine-reaction product of an aldacet, an aldacet being, as herein set forth, one of the aldehyde equilibrium products which result when acetaldehyde is put in alkali metal cyanide solution.

9. In a process for the electrodeposition of cadmium, the step comprising depositing cadmium from a cyanide-cadmium bath which contains a metal of the iron group having an atomic weight greater than fifty-eight, and an amine-reaction product of a ketaldone.

10. In a process for the electrodeposition of cadmium, the step comprising depositing cadmium from a cyanide-cadmium bath in the presence of an addition agent comprising an amine reaction product of a ketaldone.

11. In a process for the electrodeposition of cadmium, the step comprising depositing cadmium from a cyanide-cadmium bath in the presence of an addition agent comprising an amine reaction product of a carbocyclic ketaldone.

12. In a process for the electrodeposition of cadmium, the step comprising depositing cadmium from a cyanide-cadmium bath in the presence of an addition agent comprising an amine reaction product of an aliphatic ketaldone.

13. In a process for the electrodeposition of

cadmium, the step comprising depositing cadmium from a cyanide-cadmium bath in the presence of an addition agent comprising an amine reaction product of an aliphatic ketaldone which contains only carbon, hydrogen and oxygen, which has no less than two and no more than nine carbon atoms, and in which the ratio of hydrogen to oxygen is greater than that of water.

14. In a process for the electrodeposition of 10 cadmium, the step comprising depositing cadmium from a cyanide-cadmium bath in the presence of an addition agent comprising an amine reaction product of an aldacet, an aldacet being, as herein set forth, one of the aldehyde 15 equilibrium products which result when acetaldehyde is put in alkali metal cyanide solution.

15. In a process for the electrodeposition of cadmium, the step comprising depositing cadmium from a cyanide-cadmium bath in the presence of an addition agent comprising an amine reaction product of an aliphatic aldehyde selected from the group consisting of aldol, acetaldehyde, crotonaldehyde, and paraldol.

16. In a process for the electrodeposition of 25 cadmium, the step comprising depositing cadmium from a cyanide-cadmium bath in the presence of an addition agent comprising an amine reaction product of aldol.

17. In a process for the electrodeposition of 30 cadmium, the step comprising depositing cadmium from a cyanide-cadmium bath in the presence of an addition agent comprising an ethanola-amine-reaction product of an aldacet, an aldacet being, as herein set forth, one of the aldehyde 35 equilibrium products which result when acetaldehyde is put in alkali metal cyanide solution.

JOHN V. VAUGHEN.